

# United States Patent Office

2,833,649

Patented May 6, 1958

1

2,833,649

## LIGHT-SENSITIVE DIAZOTYPE MATERIAL

Oskar Süs, Wiesbaden-Biebrich, and Manfred Grundkötter, Wiesbaden, Germany, assignors, by mesne assignments, to Keuffel & Esser Co., Hoboken, N. J., a corporation of New Jersey

No Drawing. Application August 6, 1954  
Serial No. 448,393

Claims priority, application Germany August 11, 1953

12 Claims. (Cl. 96—91)

This invention is concerned with light-sensitive diazotype material. It is particularly advantageous when applied to diazotype materials of the one component or moist developing type.

Diazo compounds derived from para-phenylene diamine in which the non-diazotized amino group is secondary or tertiary have been used for the production of a light-sensitive layer on base material suitable for diazotype printing. Diazo compounds derived from para-phenylene diamine and having alkyl residues with external atom groups at the nitrogen of the un-diazotized amino group, e. g. substituted amino groups or hydroxyl groups etherified by aliphatic hydrocarbon residues, are described for this purpose in German patent specification No. 831,804 and U. S. Patent No. 2,336,309. On account of their low coupling activity, diazo compounds of this type are used particularly for the production of so-called two-component diazotype layers for dry development.

An object of the present invention is to provide an improved light-sensitive diazotype material particularly for one component or moist development.

The improved diazotype materials according to the present invention provide light sensitive diazotype material in which the light-sensitive layer includes a diazo compound of para-phenylene diamine of the general formula:



wherein

Ph is a phenylene residue which may be substituted.  
X is O, S or SO<sub>2</sub>

R<sub>1</sub> is H or an alkyl residue having 1 to 3 carbon atoms.  
R<sub>2</sub> is an aromatic residue which may be substituted.  
n is 2 or 3

The diazo compounds used in accordance with the present invention have high coupling activity, which makes them very suitable for one component, moist or semi-wet development papers. This allows the use of only slightly alkaline or even neutral developers for the production of good contrast copies, which previously was only possible when the diazo compounds of acylated p-phenylene diamines were used as the light-sensitive substance.

By introducing substituents into R<sub>2</sub>, e. g. halogen atoms, or by enlarging this residue, the coupling process during development can frequently be accelerated.

Images with deep black or brown lines are produced by the diazo compounds of this invention. The compounds are preferably applied in the form of water-soluble diazonium salts or double salts. The color depends on the azo component used. Polyhydroxy benzenes, such as 70 phloroglucinol and resorcinol are particularly suitable.

2

The shade of color can also be affected by introducing substituents into the phenylene residue which carries the diazo group. Positive substituents generally cause a lightening of the tone. Diazo compounds of this nature are suitable for the production of intermediate originals of good opacity for ultraviolet light.

The light-sensitive layers may contain the usual stabilizers in the form of inorganic or organic acids, acid salts and salts of aromatic sulphonic acids. Anti-yellowing materials, particularly thiourea and its water-soluble derivatives may also be present in the layers to improve the background of the copies after development. The light-sensitive material may be further improved to produce copies with increased contrast by incorporating suspensions of finely-divided silicon dioxide or of silicates of alkaline earth metals in the sensitizing solutions.

Known methods are used to produce the diazo compounds of this invention. For example, monoalkylated amines are used as starting material and are caused to react with the toluene-sulphonic acid esters of glycol-monoaryl-ethers or the aryl ethers of ethylene chlorhydrin or ethylene bromhydrin. The aryloxy alkylated amino benzenes thus obtained are converted to azo dyes by coupling with diazotized sulphamic acid or diazotized aniline, and from these the corresponding phenylene diamines can be obtained by reduction and can be converted in the usual manner to the diazo compounds. The amino group can also be introduced by nitrosating the tertiary bases and reducing the nitroso compounds.

The sulphur analogues are obtainable in a similar manner. In this case the thioaryl ethers of thiochlorhydrins are used as starting materials for reaction with the secondary bases.

The following is a description by way of example of methods of carrying the invention into effect. The formulae referred to are tabulated below the examples.

### Example I

To produce a coating solution, 0.1 gm. gelatine, 0.5 gm. citric acid, 2.0 gms. ammonium sulphate and 1.8 gms. of the zinc chloride double salt of N-ethyl-N-( $\beta$ -phenoxy-ethyl)-p-phenylene diamine-diazonium chloride (Formula 1) are dissolved in water and made up to 100 cc. A raw paper base material suitable for the production of photo-copying material is coated with this solution in normal manner and after drying is exposed under a transparent drawing original. The exposed paper is developed with a solution containing 2 gms. of sodium carbonate, 2.5 gms. borax, 3 gms. thiourea, 4 gms. sodium sulphate, 0.4 gm. phloroglucinol, 0.4 gm. resorcinol and 0.03 gm. saponin in 100 cc. water. The copies have dark black lines, slightly tinged with red, on a white background. They do not run and they have high contrast. The coupling speed of the diazonium chloride zinc chloride double salt used is so high that the azo dye can be developed even with a neutral to slightly acid developer (pH 7-6.5) to give sufficiently thorough development. For example, black copies with a blueish tinge are obtained with a neutral developer containing 10 gms. tertiary sodium citrate, 5 gms. sodium benzoate, 5 gms. anhydrous sodium acetate, 0.7 gm. phloroglucinol, 0.03 gm. acetoacetic anilide and 0.03 gm. saponine dissolved in water to 100 cc.

The diazo compound of Formula 1 is produced either by nitrosating N - ethyl - N - ( $\beta$ -phenoxy-ethyl)-aniline (Clemo and Perkin, Journal of the Chemical Society 121 (1922), 645) reducing the nitroso compound and diazotizing the reduction product or by reducing the azo dyestuff obtained from the above-mentioned N-tertiary

aniline by the coupling on diazotized sulphanilic acid and then diazotizing in known manner.

For example, 52 gms. N-ethyl-N-( $\beta$ -phenoxyethyl)-aniline are suspended in 520 cc. of 30% sulphuric acid and nitrosated with 40 cc. of 33% sodium nitrite solution. The nitroso compound is reduced by the introduction of zinc dust at 25-30° C. The resulting sulphuric acid solution is mixed with 150 gms. ice and diazotized with 35 cc. of 33% sodium nitrite solution. The diazo compound first comes out as an oil. 60 gms. sodium chloride are added and the reaction mixture is stirred until the zinc chloride double salt appears in the form of crystals which are filtered off with vacuum. The raw product is purified by dissolving in 1500 cc. water at 50° C., filtering over animal charcoal and separating out the zinc chloride double salt by adding 140 gms. sodium chloride.

*Example II*

1.7 gms. of the zinc chloride double salt of N-ethyl-N-( $\beta$ -phenyl-mercapto-ethyl)-p-phenylene diamine-diazonium chloride (Formula 2) is dissolved in water with 0.5 gm. tartaric acid, 0.5 gm. aluminum sulphate and 6.0 gms. 1:3:6-naphthalene trisulphonic acid sodium salt and made up to 100 cc. Paper is coated in known manner with this solution and exposed under an original after drying. Development of the exposed paper is carried out with the alkaline developer described in Example I. Copies are obtained with very strong deep black images with no tendency to run. The contrast is even better than with the copies obtained in the manner described in Example I, and the shade is rather more neutral, so that the half-tones show as pure blacks in the copies.

Equally good results are obtained by using for producing the light-sensitive layer the zinc chloride double salts of the diazonium salts of other paraphenylenediamine derivatives of the general formula stated above, for example the diazonium chlorides of Formulae 3-12:

4. N-ethyl-N-[ $\beta$ -(2:4-dichloro-phenoxyethyl)-p-phenylene diamine-diazonium chloride



Boiling point of the corresponding para-phenylene diamine (° C.)

266-270° at 19 mm.

5. N-ethyl-N-[ $\beta$ -(2-methoxy-phenoxyethyl)-p-phenylene diamine-diazonium chloride



260-265° at 15 mm.

6. N-ethyl-N-[ $\beta$ -naphthoxy-( $\alpha$ -ethyl)-p-phenylene diamine-diazonium chloride



248-250° at 2 mm.

7. N-methyl-N-[ $\beta$ -phenoxyethyl]-p-phenylene diamine-diazonium chloride



238-241° at 15 mm.

8. N-propyl-N-[ $\beta$ -phenoxyethyl]-p-phenylene diamine-diazonium chloride



255-260° at 18 mm.

65. 9. 1-(N-ethyl-N-[ $\beta$ -phenoxyethyl])-3-methyl-1:4-diamino benzene-diazonium chloride



205-207° at 3 mm.

70

10. 1-(N-ethyl-N-[ $\beta$ -phenoxyethyl])-3-methyl-1:4-diamino benzene-diazonium chloride



The diazo compound is used in the form of the stannic chloride double salt.

10. N-[ $\beta$ -phenoxyethyl]-p-phenylene diamine-diazonium chloride



Boiling point of the corresponding para-phenylene diamine ( $^{\circ}\text{C}$ )

208-213 $^{\circ}$  at 16 mm.

11. N-ethyl-N-[ $\beta$ -phenyl-sulphonyl-ethyl]-p-phenylene diamine-diazonium chloride



cannot be distilled without decomposition.

12. N-ethyl-N-( $\gamma$ -phenoxypropyl)-p-phenylene-diamine-diazonium chloride



220-223 $^{\circ}$  at 1 mm.

To produce N - ethyl - N( $\beta$  - phenyl - sulphonyl-ethyl) - p - phenylene - diamine, phenyl -  $\beta$  - chloorethyl sulphone is reacted with ethyl aniline in the presence of copper at 120 $^{\circ}\text{C}$ . The reaction product is then treated according to the instructions in Example I.

Having now particularly described the invention, what we claim is:

1. Light sensitive diazotype material for development by the semi-wet process comprising a base material coated with a light-sensitive layer including a diazo compound of a para-phenylene diamine of the general formula:



wherein

Ph is a phenylene radical

X is selected from the group consisting of O, S and  $\text{SO}_2$   
 $\text{R}_1$  is selected from the group consisting of H and alkyl radicals having 1 to 3 carbon atoms

$\text{R}_2$  is an aromatic radical directly attached to X by a carbon atom of the aromatic ring

n is selected from the group consisting of 2 and 3

2. Light sensitive diazotype material for development by the semi-wet process comprising a base material coated with a light-sensitive layer including a diazo compound of a para-phenylene diamine of the general formula:



wherein

Ph is a phenylene radical substituted by a substituent selected from the group consisting of alkyl groups and alkoxy groups

X is selected from the group consisting of O, S and  $\text{SO}_2$   
 $\text{R}_1$  is selected from the group consisting of H and alkyl radicals having 1 to 3 carbon atoms

$\text{R}_2$  is an aromatic radical directly attached to X by a carbon atom of the aromatic ring  
n is selected from the group consisting of 2 and 3

3. Light sensitive diazotype material for development by the semi-wet process comprising a base material coated with a light sensitive layer including a diazo compound of a para-phenylene diamine of the general formula:



wherein

Ph is a phenylene radical substituted by a substituent selected from the group consisting of alkyl groups and alkoxy groups

20 X is selected from the group consisting of O, S and  $\text{SO}_2$   
 $\text{R}_1$  is selected from the group consisting of H and alkyl radicals having 1 to 3 carbon atoms

$\text{R}_2$  is an aromatic radical directly attached to X by a carbon atom of the aromatic ring and substituted by a substituent selected from the group consisting of halide atoms, alkyl groups and alkoxy groups

n is selected from the group consisting of 2 and 3

4. Light sensitive diazotype material for development by the semi-wet process comprising a base material coated with a light-sensitive layer including a diazo compound of a para-phenylene diamine of the general formula:



wherein

Ph is a phenylene radical

40 X is selected from the group consisting of O, S and  $\text{SO}_2$   
 $\text{R}_1$  is selected from the group consisting of H and alkyl radicals having 1 to 3 carbon atoms

$\text{R}_2$  is an aromatic radical directly attached to X by a carbon atom of the aromatic ring and substituted by a substituent selected from the group consisting of halide atoms, alkyl groups and alkoxy groups

n is selected from the group consisting of 2 and 3

5. Light sensitive diazotype material for development by the semi-wet process comprising a base material coated with a light-sensitive layer including a diazo compound of a para-phenylene diamine of the general formula:



wherein

Ph is a phenylene radical

60 X is selected from the group consisting of O, S and  $\text{SO}_2$   
 $\text{R}_1$  is selected from the group consisting of H and alkyl radicals having 1 to 3 carbon atoms

$\text{R}_2$  is an aromatic radical directly attached to X by a carbon atom of the aromatic ring and substituted by halogen atoms

n is selected from the group consisting of 2 and 3

6. Light sensitive diazotype material for development by the semi-wet process comprising a base material coated with a light-sensitive layer including a stabilizer and a diazo compound of a para-phenylene diamine of the general formula:



wherein

Ph is a phenylene radical

X is selected from the group consisting of O, S and SO<sub>2</sub>

R<sub>1</sub> is selected from the group consisting of H and alkyl radicals having 1 to 3 carbon atoms

R<sub>2</sub> is an aromatic radical directly attached to X by a carbon atom of the aromatic ring

n is selected from the group consisting of 2 and 3

7. Light sensitive diazotype material for development by the semi-wet process comprising a base material coated with a light-sensitive layer including an anti-yellowing material and a diazo compound of a para-phenylene diamine of the general formula:



wherein

Ph is a phenylene radical

X is selected from the group consisting of O, S and SO<sub>2</sub>

R<sub>1</sub> is selected from the group consisting of H and alkyl radicals having 1 to 3 carbon atoms

R<sub>2</sub> is an aromatic radical directly attached to X by a carbon atom of the aromatic ring

n is selected from the group consisting of 2 and 3

8. Light sensitive diazotype material comprising a base material coated with a light-sensitive layer including N-

ethyl-N-( $\beta$ -phenoxyethyl)-p-phenylene diamine-diazonium chloride.

9. Light sensitive diazotype material comprising a base material coated with a light sensitive layer including N-ethyl-N-( $\beta$ -phenyl-mercapto-ethyl)-p-phenylene diamine-diazonium chloride.

10. Light sensitive diazotype material comprising a base material coated with a light sensitive layer including N-ethyl-N-[ $\beta$ -(p-chlor)-phenoxyethyl - p - phenylene diamine-diazonium chloride.

11. Light sensitive diazotype material comprising a base material coated with a light sensitive layer including N-ethyl-N-[ $\beta$ -(2-methoxy)-phenoxyethyl]-p-phenylene diamine-diazonium chloride.

12. Light sensitive diazotype material comprising a base material coated with a light sensitive layer including N-methyl-N-[ $\beta$ -phenoxyethyl]-p-phenylene diamine-diazonium chloride.

20 References Cited in the file of this patent

UNITED STATES PATENTS

2,542,566 Pedlow et al. ----- Feb. 20, 1951  
2,551,133 Jennings et al. ----- May 1, 1951

25

FOREIGN PATENTS

507,153 Great Britain ----- June 9, 1939  
831,804 Germany ----- Feb. 18, 1952